

## UNITED STATES PATENT OFFICE

ULRICH DIEM-BERNET, OF SPEICHER, SWITZERLAND  
MANUFACTURE OF LIGHT-SENSITIVE FILMS

No Drawing. Application filed May 17, 1927, Serial No. 192,163, and in Switzerland and Germany  
May 21, 1926.

It is known to produce a light sensitive film having no sensitive coating from cellulose-sodium-xanthate (viscose) and having the sensitizing agent within the film material. Such known film is prepared like the sensitive salt papers by treating finished films hitherto mainly used as a transparent packing material, in one or more baths of water containing solutions of sensitizers and impregnating them thus with light sensitive materials. In each of these baths the film swells and extends in every direction and subsequently contracts during the drying operation, whereby the original dimensions are only reached under the most favorable circumstances. The divergence from the original size is the greater, the larger the number of baths through which the film has to be passed.

This is a disadvantage which renders such films unsuitable for certain photographic purposes and particularly for the cinematographic art.

The present process has for its object to produce from viscose light sensitive negative and dia-positive films which have no sensitive coating but are sensitized within the body of the film and which are subjected to much less variations in tension than the impregnated film having no coating and produced by the hitherto known processes. In contradistinction to the known process according to which the film, which has been manufactured (i. e., cast, coagulated, washed and dried) ready for sale without additions of sensitizers, is impregnated with sensitizing materials later on, the novel process consists in sensitizing the film mass already during the manufacture i. e., at least before the ultimate and complete drying of the film, while the latter is still moist and therefore in its swollen condition. This is effected in that either all the sensitizing agents or at least one of the components used for sensitizing purposes is incorporated in the film mass, for example after a purification bath with which the cast but not yet finished film is treated, preferably after the last purification or washing bath. Preferably, simultaneously or in a subsequent step of the process, by the addition of tanning substances,

a further reduction of the susceptibility towards water and eventually of the inflammability of the film mass may be obtained.

In producing such a light sensitive film from viscose and which has no sensitive coating the present process may be carried into effect by imbuing the film, for example after a purifying bath with for instance a ferric salt solution (ammonium-ferric-citrate). The sensitizing of the film mass with a silver halid may be effected by first adding to the film the halogen source (for instance sodium-chloride, ammonium bromide), whereupon the film charged with this component is either directly or after superficial drying impregnated with a silver solution for instance with silver nitrate in order to cause the formation of silver halid.

A tanning of the film mass may be caused either during the casting of the film in a bath containing for instance alum, or ammonium salts, or it is caused subsequently to the casting of the film by smoking the sensitized film, for instance in formaldehyde vapours.

The light sensitive film without a coating manufactured in the above manner gives a more perfect saturation of the film mass than the hitherto known impregnating process. Moreover the improved process permits in a better manner than heretofore to influence important mechanical qualities of the film such as hardness, flexibility and the like, further the inflammability of the finished product as well as to obtain the necessary sterility and purity of the film mass required for special photographic purposes.

It is a particular object of the present process to produce a completely transparent light sensitive cellulose film having no coating which even in the sensitized state is transparent like glass and which presents a considerable technical progress for the special purposes of making reflex copies. (Player-type). The hitherto known processes are limited to soaked hygroscopic cellulose films in the manner of salt papers or to impregnation by means of baths containing silver compounds to cause the formation of silver chlorid or silver bromide within the body of the film whereby a certain sensitivity but not

a most perfect transparency is obtained at the same time. The present process on the contrary intends and permits the production of negative and positive films having no coatings which not only have a good sensitivity but are at the same time completely transparent like glass and which, owing to their extraordinary transparency absorb the reflected light much less than the hitherto known copying material 10 and which are therefore particularly suitable for the purposes of the reflex copy.

The more or less pronounced dullness and cloudiness of the hitherto known films made of hygroscopic cellulose by soaking them in 15 solutions of silver salts are due to the insufficient penetration of the sensitizing solutions into the interior of the film and by the precipitation of silver salts in zones in which unevenly swollen layers contact, further they 20 are due to precipitation effects between silver and chlorine of a smaller degree of dispersion as well as to such exceeding the optimum of the concentration in silver. The manufacture of sensitized films that are as clear 25 as glass is made according to the present process in the following manner: After the film mass has been completely penetrated by a suitable chlorine compound, for instance 4% sodium chloride solution, the impregnation 30 with the solution of silver salt for instance with a 10% solution of silver nitrate, is only then caused directly, if the chlorinated film mass is still as clear as glass after drying and if it does not opalize. The impregnation 35 with silver salts shall further only last as long as no formation of larger agglomerations occurs. If the film mass looks dull in any way after the chlorination a longer or shorter water bath has to be arranged before 40 the impregnation with the solution of silver, this bath has also to be used if a stronger solution of silver salt has to be applied.

The manufacture of the sensitized films, which are as clear as glass, involves a great 45 technical progress and is of the utmost importance for making reflex copies. The use of these novel copying films presents also a great advantage in producing completely transparent and at the same time true to scale 50 copies and diapositives, as such sensitive films which have no coating and are as transparent as glass permit a simpler and quicker treatment in the developing and fixing process and therefore they are less subject to the 55 swelling influence of water.

I claim:

1. A process for producing light-sensitive negative and positive films having no coating, which consists in incorporating sensitizing agents in the film mass of viscose during 60 the manufacture of the film material.

2. A process for producing light-sensitive negative and positive films having no coating, which consists in incorporating sensitizing agents in a film mass of viscose imme- 65

diate after the coagulation of the film material and before final drying.

3. A process for producing light-sensitive negative and positive films having no coating, which consists in incorporating sensitizing agents in a film mass of viscose immediately after the coagulation and the washing of the film material and before completion of the film by drying. 70

4. A process for producing light-sensitive negative and positive films having no coating, which consists in incorporating at least one component of the sensitizer in a film mass of viscose during the manufacture of the film material and before final drying of the 75 film. 80

5. A process for producing light-sensitive negative and positive films having no coating, which consists in incorporating a silver salt in a film mass of viscose during the manufacture of the film material. 85

6. A process for producing light-sensitive negative and positive films having no coating, which consists in incorporating at least one component of the sensitizer in a film mass 90 of viscose during the manufacture of the film material, the concentration of the sensitizer and the manner of incorporation being so chosen that the film mass remains perfectly transparent. 95

7. A process for producing light-sensitive negative and diapositive cellulosic films from viscose, having no coating, and having the sensitizer incorporated within the body of the film, which consists in incorporating 100 sensitizing agents in the film mass during the manufacture of the film while the latter is still in its swelled condition and before it is ultimately dried.

8. A process for producing light-sensitive negative and diapositive cellulosic films from viscose, having no coating, which consists in incorporating at least one component of the sensitizer in the film mass during the manufacture of the film while the latter is still in 105 its swelled condition before it is ultimately dried. 110

9. A process for producing light-sensitive negative and diapositive cellulosic films from viscose, having no coating, which consists in incorporating at least one component of the sensitizer in the film mass during the manufacture of the film, the concentration of the sensitizer and the manner of incorporation being so chosen that the film mass remains 115 perfectly transparent. 120

10. A process for producing light-sensitive negative and diapositive cellulosic films from viscose, having no coating, and having the sensitizer incorporated within the body of 125 the film, substantially as described.

11. A process for producing viscose photographic films having no coating, which comprises introducing into the film during its manufacture and while in a swollen condi- 130

tion, a sensitizing agent, the film being hardened by a hardening agent.

12. A glass-clear grain-free viscose photographic film, sensitized in its body and substantially free from subsequent alteration upon development and spots due to opalescence and uneven charging of sensitizer resulting from uneven swelling of the film.

5 In testimony whereof, I have signed my  
10 name to this specification.

ULRICH DIEM-BERNET.

15

20

25

30

35

40

45

50

55

60

65